

## UNITED STATES PATENT OFFICE

1,972,137

## TREATMENT OF TEXTILE MATERIALS

George Holland Ellis, Spondon, near Derby, England, assignor to Celanese Corporation of America, a corporation of Delaware

No Drawing. Application March 26, 1930, Serial No. 439,264. In Great Britain April 29, 1929

17 Claims. (Cl. 8—5)

This invention relates to the production of coloured pattern effects on fabrics or other textile materials.

In the colouration of textile materials, particularly in the case of fabrics, it is frequently required to produce white or coloured pattern effects on a coloured ground, and such effects are commonly produced by dyeing or otherwise colouring the fabric and then removing or changing the colour of selected portions by the application of the so-called discharging agents which may destroy the colouring matter or may convert it into an uncoloured or differently coloured compound or into a form in which it is easily removed from the fabric by washing. Thus certain colouring matters can be discharged by the application of reducing agents, certain others by application of oxidizing agents, while some can be discharged by either oxidizing or reducing agents. If the discharging agent is mixed with a colouring matter which is not destroyed thereby but which has affinity for the fabric or other material to be treated it is possible not only to remove the ground colour in selected places but to substitute another colour therefor; in this manner the so-called coloured discharges may be obtained.

The production of such white and coloured discharge effects on materials made of or containing cellulose acetate or other organic acid esters of cellulose or cellulose ethers has been attended with some difficulty but very good discharge effects can be produced on such materials by the chlorate discharge process described in British Patent No. 312,655, or by the use of chromates as described in U. S. Patent No. 1,925,178 or by the use of other oxidizing agents as described in U. S. Patent No. 1,905,346.

Valuable white or coloured discharge effects can also be obtained on materials made of or containing cellulose acetate or other organic acid esters or ethers of cellulose by the processes described in United States Patent No. 1,922,927. According to this specification discharge effects are obtained by applying to the material a diazotizable amine or colouring matter, then printing a discharging agent which may be an oxidizing or a reducing agent, and thereafter diazotizing and combining with a coupling component which may be applied simultaneously with or separately from the diazotizable compound.

According to the present invention in the production of white or coloured discharge effects on textile materials, the material is impregnated

with a substance having an acid reaction prior to the application of the discharging agent.

The employment of a substance of acid reaction in this manner greatly facilitates the action of the discharging agent, particularly when operating on materials made of or containing cellulose acetate or other cellulose esters, or cellulose ethers. Moreover, particularly in the cases where reducing agents are employed as the discharging agent, the presence of the acid substance in the material prevents the edges of the pattern from becoming blurred or "haloed" due to the spreading of the discharging agent beyond the desired boundary lines.

The incorporation of a substance of acid reaction in the material in accordance with the invention is not only applicable in those cases where discharge of a colouring matter already present in the material is to be effected but is equally applicable where a diazotizable compound is to be discharged locally, prior to diazotization and development, in the manner described in the aforesaid United States Patent No. 1,922,927.

As substances of acid reaction which may be employed according to the invention may be mentioned organic acids, particularly organic carboxylic acids, preferably such as are only volatile with difficulty, for example oxalic acid, tartaric acid, or citric acid. Other acids which may be used are for example salicylic acid, benzoic acid, a naphthoic acid, and sulphonic acids such as those of benzene, phenol, naphthalene, or the naphthols. The invention is not however limited to the use of organic acids since other substances having an acidic reaction, for instance acid salts or salts which have an acid reaction, for example aluminium sulphate or zinc sulphate, may be employed. Care should be taken that the acid substance is not of such nature or is not used under such conditions as would lead to damage to the textile material under treatment.

The substances of acid reaction may be applied to dyed materials in any convenient manner, for example by passing the materials through a solution thereof in water or by padding them with such a solution. The latter method is particularly convenient in the case of woven fabrics. After the impregnation with the acid substance the materials are preferably dried prior to the application of the discharging agent.

As discharging agents may be used any of those commonly used in the art of textile printing, for example reducing agents such as hydrosulphites or formaldehyde sulphoxylates, especially sodium formaldehyde sulphoxylates, or oxidizing agents

such as chlorates or chromates. They will in general be applied to the textile materials in admixture with thickening agents designed to give them the physical properties necessary in a preparation which is to be applied to a fabric by printing or other mode of local application. Further the discharging preparation may contain catalytic or other substances which assist the discharging action on the dyed material; thus a reducing discharge preparation may contain anthraquinone, and an oxidizing discharge preparation may contain an acidic substance and/or oxidation catalysts such as salts of iron, prussiates, or salts of vanadium. When it is required to produce discharge effects upon materials made of or containing cellulose esters or ethers according to the process of the invention the action of the discharging preparation may frequently be intensified by incorporating therein a swelling agent for the said cellulose derivative, for example a sulphocyanide or alcohol, e. g. in the form of methylated spirit.

Coloured discharges can be produced according to the invention by incorporating in the discharge preparations colouring matters which are not destroyed thereby under the working conditions and which have affinity for or can be fixed on the textile material under treatment. Vat dyestuffs, certain basic dyestuffs such as methylene blue or rhodamine 6 G extra, and certain mordant dyestuffs are particularly suitable for incorporation in reducing discharges. For use in oxidizing discharges may be mentioned the resistant colouring matters referred to in British Patent No. 312,655, for example colouring matters of the mineral pigment type such as chrome yellow, lemon chrome yellow, Guignet's green, and vermillion, organic dyestuffs of the pigment type (insoluble in water but soluble in oils, fats, soaps or the like) e. g. resistant vat dyes of the anthraquinone series or the following insoluble azo dyes:— m-nitraniline naphthol A S, p-nitraniline- $\beta$ -naphthol or naphthol A S, and p-nitro-o-toluidine- $\beta$ -naphthol or naphthol A S, certain basic dyestuffs for example methylene blue and rhodamine 6 G extra.

For colouring oxidizing discharges intended for application to materials made of or containing cellulose esters or ethers, many of the dyestuffs normally employed for colouring such materials are very suitable. For example nitro diarylamine colouring matters and aminoanthraquinone colouring matters can be used very successfully. Care should be exercised however in the choice of dyestuffs of the  $\alpha$ -aminoanthraquinone series since some members of this class having a substituent, particularly hydroxyl or amino, in the para position to the  $\alpha$ -amino group are insufficiently resistant to the action of oxidizing discharge preparations.

Other colouring matters which have been found useful, particularly for incorporation in oxidizing discharge preparations, are the acidyl aminoanthraquinones whether simple acidylamino compounds or containing in addition to acidylamino groups other substituent groups or atoms such as hydroxyl groups, alkoxy groups, and halogen atoms. Of this group of colouring matters the aliphatic acidyl aminoanthraquinones are of especial interest for use in colouring oxidizing discharge preparations for application to cellulose ester or ether materials owing to their good affinity for such materials; the following are examples of such aliphatic acidyl aminoanthraquinones and the colourations yielded by

them when applied to cellulose ester or ether materials:—

|                                                                   |                      |    |
|-------------------------------------------------------------------|----------------------|----|
| 1-acetyl amino-anthraquinone                                      | Yellow               |    |
| 1-propionyl amino-anthraquinone                                   | Yellow               |    |
| 1 - acetyl amino - 2 - methyl - anthraquinone                     | Yellow (less green)  | 80 |
| 1 - acetyl amino - 4 - hydroxy - anthraquinone                    | Golden orange        |    |
| 1 - propionyl amino - 4 - methoxy - anthraquinone                 | Golden yellow        |    |
| 1 : 4 - (propionyl amino) - anthraquinone                         | Red                  |    |
| 1 - methy lamino - 4 - acetyl amino-anthraquinone                 | Reddish violet       | 85 |
| 1 : 4 - di (acetyl ethyl amino) - anthraquinone                   | Red                  |    |
| 1 : 5 - di (acetyl amino) - 4 : 8 - dihydroxy-anthraquinone       | Red                  |    |
| 1 - propionylmethylamino - 4 : 5 - dihydroxy-anthraquinone        | Red                  |    |
| 1 : 5 - di (acetyl methylamino) - 5 : 6 - dihydroxy-anthraquinone | Violet               | 90 |
| 2-propionylamino-anthraquinone                                    | Pale greenish yellow |    |

The above aliphatic acidylaminoanthraquinones may be prepared by treating the corresponding aminoanthraquinone or aminoanthraquinone derivative with the acid anhydride, acetic or propionic, in acetic acid solution.

The dyestuffs in the coloured discharge preparations may if desired or requisite be applied in conjunction with a fixing agent or agents, for example with albumen in the case of pigment dyestuffs and with mordants in the case of mordant or basic dyestuffs. Vat dyestuffs may be applied in the form of the esters of their leuco compounds.

The application of the discharge preparations to the dyed material, after incorporating a substance of acid reaction therein, may be effected in any desired manner, for example by machine or hand-block printing, stencilling, spraying or the like.

As previously indicated the presence of the substance of acid reaction in the dyed material greatly facilitates the action of the discharging agent, so much so, that the discharging action frequently takes place on simply drying the material after applying the agent and without the subsequent ageing or steaming operation commonly practised in the art. In the production of coloured discharges however, steaming is often desirable to fix satisfactorily the colouring matter on the discharged portions of the materials. Where such is the case and the said colouring matter is insufficiently resistant to the combined action of steam, discharging agent, and an acid, the last mentioned may be neutralized prior to steaming, for example by treatment with gaseous ammonia or with a dilute solution of ammonia, soda ash, or other alkali. Especially useful results are obtained as previously indicated when the new process is applied to the treatment of textile materials made of or containing cellulose acetate or other cellulose esters, or cellulose ethers. For example, valuable coloured discharge effects in great variety can readily be produced upon such materials coloured with dischargeable dyestuffs of the galloycyanine series or basic dyestuffs of the diaryl-methane, triaryl-methane, thiazine, oxazine, azine, or xanthene series. For instance, material dyed with one or more of the aforementioned colouring matters may be impregnated with a substance having an acid reaction and an oxidizing discharge preparation containing a colouring matter of the nitro diarylamine or aminoanthraquinone series applied by printing or other mode of local application. Discharge of the ground colouration may be effected without steaming, for example by drying the printed fabric by means of warm or hot air or heated surfaces such as cylinders, but, in order to fix prop-

115

120

125

130

135

140

145

150

erly the colouring matter on the discharged portions of the material, the latter may be subsequently steamed after treatment with an alkali, for example, gaseous ammonia or dilute aqueous alkali.

The invention is applicable to the production of discharge effects on textile materials of all kinds, for example materials made of or containing cotton, silk, or artificial silk whether of the 10 regenerated cellulose type or of the type made from cellulose esters, for example cellulose acetate, formate, propionate, or butyrate, or the products obtained by the treatment of alkalinized cellulose with esterifying agents (e. g. the product known as "immunized cotton" obtained with p-toluene-sulphochloride) or made from cellulose ethers, for instance methyl, ethyl, or benzyl cellulose or the corresponding condensation products of cellulose and glycols or other polyhydric 20 alcohols. Mixed materials made from two or more types of textile filaments, threads or yarns may also be treated in accordance with the invention.

The following examples show the best way 25 known to us for carrying the invention into effect but are not intended to limit it in any way.

#### Example 1

A fabric woven from cellulose acetate yarns is 30 dyed by known methods with 5% of its weight of violet P. D. H. (Colour Index No. 893). After dyeing the fabric is soaped lightly, rinsed and dried. It is then padded in a 5% solution of 35 oxalic acid, squeezing to hold about its own weight of liquor, and dried. The acid-padded fabric is printed with a discharge paste composed as follows:—

|                           | Grams |
|---------------------------|-------|
| Gum arabic 1:1            | 450   |
| 40 Aluminium sulphate 1:1 | 190   |
| Sodium chlorate           | 90    |
| Potassium ferricyanide    | 30    |
| Water                     | 240   |
|                           | 1000  |

The printed fabric is dried hard, either in a 45 hot chamber or on steam heated drums, after which it is washed free from acid in water and finally soaped lightly. A white pattern on a deep blue-violet ground is thus obtained.

#### Example 2

A fabric woven from cellulose acetate yarns is 50 dyed in a dye bath of volume ratio 50:1 with 0.5% of its weight of benzene-azo-1-phenyl-3-methyl-5-pyrazolone, the dyestuff being dispersed before adding to the dye bath by heating with four times its weight of sodium sulphuricinoleate. After 55 dyeing for 1½ hours at 80° C. the material is rinsed and dried and then padded in a 5% solution of citric acid, squeezing to leave its own weight of liquor in the fabric, and again dried. It is then printed with the paste given in Example 1, dried and suitably steamed for 2 minutes 60 at 100° C. after which it is rinsed well and soaped lightly. A white pattern on a bright yellow ground is obtained.

#### Example 3

70 A woven fabric composed of cellulose acetate yarns is dyed by known methods with 0.5% of its weight of 4-nitro-benzene-azo-para - xylidine. After dyeing for 1½ hours at 80° C. the material 75 is rinsed and dried and then padded in a 5% solution of oxalic acid, being squeezed so as to

retain its own weight of pad liquor, and dried. The acid padded fabric is printed with the following discharge paste:—

|                         | Grams |      |
|-------------------------|-------|------|
| Gum arabic 1:1          | 580   | 80   |
| Zinc oxide              | 50    |      |
| Methylated spirit       | 100   |      |
| Water                   | 50    |      |
| Anthraquinone 10% paste | 70    |      |
| Formosul                | 150   | 85   |
|                         |       | 1000 |

The printed fabric is dried and suitably steamed either in the "rapid ager" or in the cottage steamer, after which it is rinsed and soaped lightly. A white pattern on a bright orange ground is obtained.

#### Example 4

A woven fabric composed of cellulose acetate 95 yarns is dyed by known methods with 0.5% of its weight of 4-nitro-2-methoxy-benzene-azo-diethylaniline and after drying it is padded in a 5% solution of benzene-sulphonic acid, being squeezed to retain about its own weight of liquor, 100 and dried. The padded fabric is printed with a paste composed as follows:—

|                         | Grams |      |
|-------------------------|-------|------|
| Gum arabic 1:1          | 500   |      |
| Ciba blue 2B. powder    | 50    | 105  |
| Anthraquinone 10% paste | 60    |      |
| Sodium hydrosulphite    | 30    |      |
| Caustic soda            | 30    |      |
| Soda ash                | 30    |      |
| Water                   | 100   | 110  |
| Methylated spirit       | 50    |      |
| Formosul                | 100   |      |
|                         |       | 1000 |

After printing the material is dried and suitably steamed either in the rapid ager or cottage steamer and oxidized in a bath of sodium dichromate for 5 minutes at 60° C. It is finally rinsed and soaped. A blue pattern on a red ground is obtained.

#### Example 5

A fabric composed of cellulose acetate yarns is dyed by a known method with 5% of its weight 125 of violet P. D. H. (Colour Index No. 893). After drying it is padded in a substance of an acid character, for instance as described in Example 1, 2, 3 or 4, and after drying is printed with a paste of the following composition:—

|                                            | Grams |      |
|--------------------------------------------|-------|------|
| Gum arabic 1:1                             | 440   |      |
| Aluminium sulphate 1:1                     | 190   |      |
| Sodium chlorate                            | 90    |      |
| Water                                      | 100   | 135  |
| 1-methylamino - 2 - methyl - anthraquinone |       |      |
| 20% aqueous paste                          | 150   |      |
| Potassium ferricyanide                     | 30    |      |
|                                            |       | 1000 |

After printing the fabric is dried on steam heated drums and then neutralized either by gassing with ammonia in a suitable apparatus or padding in an aqueous solution of an alkaline character, until there is no acid reaction, after which it is dried and steamed for 15 minutes at 5 lbs. pressure in the "cottage" steamer. The material is then rinsed and soaped lightly. A bright red pattern on a deep blue-violet ground is thus obtained.

150

*Example 6*

A woven fabric composed of cellulose acetate yarns is dyed by a known method with 3% of its weight of crystal violet (Colour Index No. 681) and after dyeing is padded in a substance of an acid nature, for instance as described in Examples 1, 2, 3 or 4. The material, after drying, is printed with a printing paste composed as follows:

|                                               | Grams |  |
|-----------------------------------------------|-------|--|
| 10 Gum arabic 1:1                             | 440   |  |
| Aluminium sulphate 1:1                        | 190   |  |
| Sodium chlorate                               | 90    |  |
| 15 Water                                      | 100   |  |
| 2:4 - dinitro - diphenylamine 20% water paste | 150   |  |
| Potassium ferricyanide                        | 30    |  |
|                                               | 1000  |  |

20 After printing the fabric is dried, neutralized with alkali, steamed in the cottage steamer and finished as described in Example 5. A brilliant yellow pattern on a violet ground is thus obtained.

*Example 7*

A cellulose acetate woven fabric is dyed by a known method with 3% of its weight of methylene blue (Colour Index No. 922) and after dyeing is padded in a substance of an acid character as in Examples 5 and 6. After drying the material is printed with a printing paste composed as follows:

|                                                               | Grams |  |
|---------------------------------------------------------------|-------|--|
| 35 Gum arabic 1:1                                             | 440   |  |
| Aluminium sulphate 1:1                                        | 190   |  |
| Water                                                         | 100   |  |
| Sodium chlorate                                               | 90    |  |
| 4-chlor-2-nitro-4' - ethoxy - diphenylamine (20% water paste) | 150   |  |
| 40 Potassium ferricyanide                                     | 30    |  |
|                                                               | 1000  |  |

45 After printing the fabric is dried, neutralized with a substance of an alkaline nature as described in Examples 5 and 6, steamed, rinsed and soaped. A bright orange design on a blue ground is obtained.

*Example 8*

50 A fabric composed of silk yarns is dyed by a known method with 3% of its weight of setoglaucone (Colour Index No. 658) and after drying is padded in a solution of a substance of an acid character as in Example 7. After drying, the material is printed with a printing paste composed as follows:

|                | Grams |  |
|----------------|-------|--|
| Gum arabic 1:1 | 650   |  |
| Zinc oxide     | 50    |  |
| 60 Water       | 150   |  |
| Formosul       | 150   |  |
|                | 1000  |  |

65 The printed fabric is dried and suitably steamed either in the rapid ager or in the cottage steamer, after which it is rinsed and soaped lightly. A white pattern on a turquoise blue ground is obtained.

*Example 9*

70 A woven fabric composed of cotton yarns is dyed by known methods with 2% of its weight of chlorazol sky blue F. F. (Colour Index No. 618) and after drying is padded in a 2% solution of citric acid, squeezing to leave its own weight of

liquor in the fabric, and carefully dried. The acid padded fabric is printed with the following discharge paste:

|                | Grams |    |
|----------------|-------|----|
| Gum arabic 1:1 | 650   | 80 |
| Zinc oxide     | 50    |    |
| Water          | 150   |    |
| Formosul       | 150   |    |
|                | 1000  | 85 |

The printed fabric is dried and suitably steamed either in the rapid ager or in the cottage steamer, after which it is rinsed and soaped lightly. A white pattern on a bright blue ground is obtained.

What I claim and desire to secure by Letters Patent is:

1. In the production of discharge effects on textile materials, impregnating the materials with a substantially non-volatile substance having an acid reaction and drying the same prior to the application of the discharging agent.

2. In the production of discharge effects on textile materials comprising an organic derivative of cellulose, impregnating the materials with a substantially non-volatile organic acid and drying the same prior to the application of the discharging agent.

3. In the production of discharge effects on textile materials comprising cellulose acetate, impregnating the materials with a substantially non-volatile organic acid and drying the same prior to the application of the discharging agent.

4. In the production of discharge effects on textile materials comprising an organic derivative of cellulose, impregnating the materials with a substantially non-volatile organic acid and drying the same prior to the application of a discharging agent which comprises an oxidizing agent.

5. Process for the production of discharge effects on textile materials, comprising impregnating the dyed materials with an aqueous solution of a substantially non-volatile substance having an acid reaction, drying the materials, and locally applying a discharging agent.

6. Process for the production of discharge effects on textile materials comprising an organic derivative of cellulose, comprising impregnating the dyed textile materials with an aqueous solution of a substantially non-volatile substance having an acid reaction, drying the materials, and locally applying a discharging agent.

7. Process for the production of discharge effects on textile materials comprising cellulose acetate, comprising impregnating the dyed textile materials with an aqueous solution of a substantially non-volatile substance having an acid reaction, drying the materials, and locally applying a discharging agent.

8. Process for the production of discharge effects on textile materials comprising an organic derivative of cellulose, comprising impregnating the dyed materials with an aqueous solution of a substantially non-volatile substance having an acid reaction, drying the materials, and locally applying an oxidizing discharge.

9. Process for the production of discharge effects on textile materials comprising cellulose acetate, comprising impregnating the dyed materials with an aqueous solution of a substantially non-volatile substance having an acid reaction, drying the materials, and locally applying an oxidizing discharge.

10. Process for the production of discharge effects on textile materials comprising an organic

derivative of cellulose, comprising impregnating the dyed materials with an aqueous solution of a substantially non-volatile organic acid, drying the materials, and locally applying an oxidizing discharge.

11. Process for the production of discharge effects on textile materials comprising cellulose acetate, comprising impregnating the dyed materials with an aqueous solution of a substantially non-volatile organic acid, drying the materials, and locally applying an oxidizing discharge.

12. Process for the production of discharge effects on textile materials comprising an organic derivative of cellulose, comprising impregnating the dyed textile materials with an aqueous solution of a substantially non-volatile organic acid, drying the materials, and locally applying an oxidizing discharge composition containing resistant

20 difficulty soluble coloring matters selected from the group consisting of the amino-anthraquinone, aliphatic acidyl-aminoanthraquinone, or nitro-diarylamine series.

13. Process for the production of discharge effects on textile materials comprising cellulose acetate, comprising impregnating the dyed textile materials with an aqueous solution of a substantially non-volatile organic acid, drying the materials, and locally applying an oxidizing discharge composition containing resistant difficultly soluble coloring matters selected from the group consisting of amino-anthraquinone, aliphatic acidyl-amino-anthraquinone, or nitro-diarylamine series.

35 14. Process for the production of discharge effects on textile materials, comprising impregnating the dyed materials with an aqueous solution of a substantially non-volatile substance having an acid reaction, drying the materials, locally ap-

plying a discharging agent containing a coloring matter resistant thereto, neutralizing the substance having an acid reaction, and then subjecting the materials to a steaming operation to fix the coloring matter.

15. Process for the production of discharge effects on textile materials comprising an organic derivative of cellulose, comprising impregnating the dyed materials with an aqueous solution of a substantially non-volatile substance having an acid reaction, drying the materials, locally applying a discharging agent containing a coloring matter resistant thereto, neutralizing the substance having an acid reaction, and then subjecting the materials to a steaming operation 90 to fix the coloring matter.

16. Process for the production of discharge effects on textile materials comprising cellulose acetate, comprising impregnating the dyed materials with an aqueous solution of a substantially non-volatile substance having an acid reaction, drying the materials, locally applying a discharging agent containing a coloring matter resistant thereto, neutralizing the substance having an acid reaction, and then subjecting the materials to a steaming operation 95 to fix the coloring matter.

17. Process for the production of discharge effects on textile materials comprising an organic derivative of cellulose, comprising impregnating the dyed materials with an aqueous solution of a substantially non-volatile organic acid, drying the materials, locally applying a discharging agent containing an oxidizing agent and a coloring matter resistant thereto, neutralizing the 105 acid, and then subjecting the materials to a steaming operation to fix the coloring matter.

GEORGE HOLLAND ELLIS.

Patent No. 1,972,137.

September 4, 1934.

GEORGE HOLLAND ELLIS.

It is hereby certified that error appears in the printed specification of the above numbered patent requiring correction as follows: Page 2, line 90, for "1:5-di" read 1:4-di; and that the said Letters Patent should be read with this correction therein that the same may conform to the record of the case in the Patent Office.

Signed and sealed this 25th day of September, A. D. 1934.

(Seal)

Leslie Frazer  
Acting Commissioner of Patents.

derivative of cellulose, comprising impregnating the dyed materials with an aqueous solution of a substantially non-volatile organic acid, drying the materials, and locally applying an oxidizing discharge.

11. Process for the production of discharge effects on textile materials comprising cellulose acetate, comprising impregnating the dyed materials with an aqueous solution of a substantially non-volatile organic acid, drying the materials, and locally applying an oxidizing discharge.

12. Process for the production of discharge effects on textile materials comprising an organic derivative of cellulose, comprising impregnating the dyed textile materials with an aqueous solution of a substantially non-volatile organic acid, drying the materials, and locally applying an oxidizing discharge composition containing resistant

20 difficulty soluble coloring matters selected from the group consisting of the amino-anthraquinone, aliphatic acidyl-aminoanthraquinone, or nitro-diarylamine series.

13. Process for the production of discharge effects on textile materials comprising cellulose acetate, comprising impregnating the dyed textile materials with an aqueous solution of a substantially non-volatile organic acid, drying the materials, and locally applying an oxidizing discharge composition containing resistant difficultly soluble coloring matters selected from the group consisting of amino-anthraquinone, aliphatic acidyl-amino-anthraquinone, or nitro-diarylamine series.

35 14. Process for the production of discharge effects on textile materials, comprising impregnating the dyed materials with an aqueous solution of a substantially non-volatile substance having an acid reaction, drying the materials, locally ap-

plying a discharging agent containing a coloring matter resistant thereto, neutralizing the substance having an acid reaction, and then subjecting the materials to a steaming operation to fix the coloring matter.

15. Process for the production of discharge effects on textile materials comprising an organic derivative of cellulose, comprising impregnating the dyed materials with an aqueous solution of a substantially non-volatile substance having an acid reaction, drying the materials, locally applying a discharging agent containing a coloring matter resistant thereto, neutralizing the substance having an acid reaction, and then subjecting the materials to a steaming operation 90 to fix the coloring matter.

16. Process for the production of discharge effects on textile materials comprising cellulose acetate, comprising impregnating the dyed materials with an aqueous solution of a substantially non-volatile substance having an acid reaction, drying the materials, locally applying a discharging agent containing a coloring matter resistant thereto, neutralizing the substance having an acid reaction, and then subjecting the materials to a steaming operation 95 to fix the coloring matter.

17. Process for the production of discharge effects on textile materials comprising an organic derivative of cellulose, comprising impregnating the dyed materials with an aqueous solution of a substantially non-volatile organic acid, drying the materials, locally applying a discharging agent containing an oxidizing agent and a coloring matter resistant thereto, neutralizing the 100 acid, and then subjecting the materials to a steaming operation to fix the coloring matter.

GEORGE HOLLAND ELLIS.

Patent No. 1,972,137.

September 4, 1934.

GEORGE HOLLAND ELLIS.

It is hereby certified that error appears in the printed specification of the above numbered patent requiring correction as follows: Page 2, line 90, for "1:5-di" read 1:4-di; and that the said Letters Patent should be read with this correction therein that the same may conform to the record of the case in the Patent Office.

Signed and sealed this 25th day of September, A. D. 1934.

(Seal)

Leslie Frazer  
Acting Commissioner of Patents.